# EUROPEAN PATENT SPECIFICATION

(11) **EP 4 493 292 B1**
(45) Date of publication and mention of the grant of the patent: **04.02.2026**
(21) Application number: 23719883.3
(22) Date of filing: 16.03.2023
(51) Int. Cl.: A63B 31/11

(54) **DIVING FIN**
TAUCHFLOSSE
PALME DE PLONGÉE

(30) Priority: 17.03.2022 SI 202200042
(43) Date of publication of application: 22.01.2025
(73) Proprietor: Kobal, Maja, 1211 Smartno pri Ljubljani (SI)
(72) Inventor: ROBINIK, Maks, 1000 Ljubljana (SI)
(74) Representative: Sveticic, Andrej
(86) International application number: PCT/IB2023/052557
(87) International publication number: WO 2023/175546

(56) References cited:
- WO-A1-2015/094127
- WO-A1-2021/207800
- CN-A- 112 976 749
- KR-B1- 101 712 751

## Description

### Field of invention

The invention relates to a diving fin.

### Prior Art

Due to a small surface area and inappropriate geometry of the human foot, diving fins were developed to provide a good thrust for the swimmer when swimming. They function in a similar way to a fish tail, but with the difference that, due to human anatomy, the thrust is generated mainly by the upward movement of the foot. In this movement, the fin blade moves upwards at an angle, pushing the water away. The fins have a rail along the longitudinal edges which helps to direct the flow of water along the fin. A wider fin blade also helps to improve the swimmer's thrust. Traditionally, diving fins were made of rubber. More recently, however, diving fins have been developed from polymer materials reinforced with carbon, glass or other high elastic modulus fibre fabrics, which provide a higher thrust force and thus greater diving fin performance.

Document WO 2021/207800 discloses a fin blade for free diving or swimming or scuba diving, which has a cross section at one end angled about a yaw, or longitudinal, axis relative to the cross section at the other end. The arrangement is such that a lateral line at a proximal end is disposed at an angle relative to a lateral line at a portion spaced from the proximal end. The advantage is that the fin blade is more closely aligned with the ergonomic complexities of the human body, such that during finning the fin blade provides greater comfort and/or propulsion. A fin blade is also described which includes a reinforced zone in one portion of the fin blade, such that one portion of the blade at the distal end is relatively increased in flexibility to provide a catch zone at one portion of the distal end of the fin blade.

Document KR101712751B1 discloses a diving fin comprising all the technical features set out in the preamble of claim 1.

### Technical problem

The technical problem is how to further increase the efficiency of diving fins. A more efficient diving fin means a better thrust for the swimmer for the same effort input, or the same thrust for the swimmer for less effort input.

### Solution to the technical Problem

The relative terms such as distal, proximal etc. are defined with respect to the user when the diving fin is in use.

The technical problem is solved by a diving fin according to claim 1 that comprises:
a foot portion and
a fin blade connected to the foot portion at its distal end, the fin blade comprising two support layers extending along the entire length of the fin blade and a plurality of inner layers between the two support layers extending from the proximal end of the blade towards the distal end over at least a portion of the longitudinal dimension of the fin blade, each support layer and inner layer comprising resin-impregnated fibres, wherein, at least in the support layers, a ratio between the number of fibres per length unit oriented in the longitudinal direction and the number of fibres per length unit oriented in the transverse direction of the diving fin is at least 1.5.

The advantage of the diving fin according to the invention over known diving fins is the increased efficiency of the diving fin. The diving fin therefore enhances the kick, allowing faster swimming.
Figure 1: Diving fin
Figure 2: Blade layers of the diving fin
Figure 3: Wavy fin blade

The invention is described in more detail hereinbelow.

The technical problem is solved by a diving fin 1 that comprises:
a foot portion 2 and
a fin blade 3 connected to the foot portion 2 at its distal end, the fin blade 3 comprising two support layers 4 extending along the entire length of the fin blade and a plurality of inner layers 5 between the two support layers extending from the proximal end of the blade towards the distal end over at least a portion of the longitudinal dimension of the fin blade, each support layer 4 and inner layer 5 comprising resin-impregnated fibres,
wherein, at least in the support layers 4, a ratio between the number of fibres per length unit oriented in the longitudinal direction and the number of fibres per length unit oriented in the transverse direction of the diving fin is at least 1.5.

The technical effect of increased efficiency of the fin occurs if the number of fibres per length unit oriented in the longitudinal direction of the diving fin is greater than the number of fibres per length unit oriented in the transverse direction of the diving fin, but the effect is in fact noticeable if the ratio between the number of fibres per length unit oriented in the longitudinal direction and the number of fibres oriented in the transverse direction of the diving fin is 1.5. If the ratio between the number of fibres per length unit oriented in the longitudinal direction and the number of fibres oriented in the transverse direction of the diving fin is 9 or greater, the efficiency of the diving fin is greater, but this has a negative impact on the mechanical strength of the diving fin in the transverse direction. The most preferred embodiment is the one, in which the ratio between the number of fibres per length unit oriented in the longitudinal direction and the number of fibres oriented in the transverse direction of the diving fin is 2 to 4.

The diving fin may further comprise two protective layers 6 disposed on the outside of each of the support layers. The protective layers may be formed of, for example, polyester or glass fibre felt impregnated with resin. The protective layers can also serve as carriers for graphic printing.

The fibres of the support and inner layers may be selected from carbon fibres, glass fibres or other fibres having a Young's modulus of at least 60 GPa and a tensile strength of at least 500 MPa, or combinations thereof.

The longitudinal and transverse fibres are preferably woven. Examples of suitable weaves: plain weave (80/20), twill (3/1), Basket weave, Jacquard weave, Dobby weave, etc.

Different numbers of fibres in the longitudinal and transversal directions in the fabric can be achieved in different ways. For example, a plain weave fabric can be used, wherein the threads in the longitudinal direction have a higher number of fibres than the threads in the transverse direction. Alternatively, a fabric may be used in which the threads in the longitudinal and transverse directions are the same, but the density of the longitudinal threads per length unit is greater than that of the transverse threads. It is also possible to combine the two ways, i.e. the number of fibres in the longitudinal threads is greater than in the transverse threads and the density of the longitudinal threads per length unit is greater than that of the transverse threads.

The resin can be chosen from epoxy resin, phenolic resin, bio resin or polyester resin.

The number of the inner layers may be 3 to 16, preferably 3 to 5.

The fin blade is preferably made by the infusion process, where layers of dry fibres are stacked on top of each other and then impregnated with resin. The advantage of the infusion process over the prepreg process, which uses pre-soaked fibres stacked on top of each other and then heat bonded, is that the final product is almost completely free of micrometre air bubbles, which has a positive effect on the lifetime of the fin blade. When manufacturing the fin blade, care must be taken that there is not excess resin in relation to fibres, as this can have a negative impact on the mechanical properties of the product.

However, when testing the diving fin according to the invention, it turned out that the flat fin blade according to the invention, due to dynamic loads (i.e. alternating compressive and tensile loads), makes more noise than the known diving fin, which is heard as a "clicking" sound when the diving fin is used in the water. Such sounds scare away fish, which is of course undesirable when spearfishing, watching or photographing fish. It has furthermore proved that there is no increase in noise if the fin blade is shaped in a wavy pattern with the crests of the waves in the transverse direction of the fin blade. Such a diving fin is a preferred embodiment of a diving fin according to the invention and will be described in more detail below.

According to a preferred embodiment, the fin blade is formed by a plurality of concave and convex segments 7a, 7b alternating from the proximal portion to the distal portion of the fin blade, with the crests of the concave and convex segments oriented transverse to the longitudinal direction of the fin blade. The amplitude of the successive concave and convex segments preferably decreases towards the distal end of the fin blade. The wave length of the successive concave and convex segments along the fin blade may be equal or decrease towards the distal end of the fin blade. The distal end of the diving fin may be formed flat, i.e. without concave and convex segments. The longitudinal edge of the fin blade may be provided with a rubber profile in the form of a wing to prevent the lateral flow of water when the diving fin is in use, thereby stabilising the movement of the diving fin in the swimming direction.

The performance of the diving fin was tested on a fin with three inner layers of glass fibre felt. The two support layers were made with a plain weave fabric having the same number of threads per length unit in the longitudinal and transverse directions, but with the threads having 12000 fibres in the longitudinal direction and 3000 fibres in the transverse direction.

## Claims

1. A diving fin (1) that comprises:
a foot portion (2) and
a fin blade (3) connected to the foot portion (2) at its distal end, the fin blade (3) comprising two support layers (4) extending along the entire length of the fin blade (3) and a plurality of inner layers (5) between the two support layers (4) extending from the proximal end of the blade towards the distal end over at least a portion of the longitudinal dimension of the fin blade, each support layer (4) and inner layer (5) comprising resin-impregnated fibres,
**characterised in that** at least in the support layers (4), a ratio between the number of fibres per length unit oriented substantially in the longitudinal direction and the number of fibres per length unit oriented substantially in the transverse direction of the diving fin is at least 1.5.

2. The diving fin according to claim 1, **characterized in that** the ratio between the number of fibres per length unit oriented in the longitudinal direction and the number of fibres oriented in the transverse direction of the diving fin is less than 9, preferably 2 to 4.

3. The diving fin according to claim 1 or 2, **characterized by** further comprising two protective layers (6) disposed on the outside of each of the support layers (4).

4. The diving fin according to any one of the preceding claims, **characterized in that** the fibres of the support (4) and inner (5) layers are selected from carbon fibres, glass fibres or other fibres having a Young's modulus of at least 60 GPa and a tensile strength of at least 500 MPa, or combinations thereof.

5. The diving fin according to any one of the preceding claims, **characterized in that** the support layers (4) are formed of a plain weave fabric, wherein the threads in the longitudinal direction have a higher number of fibres than the threads in the transverse direction.

6. The diving fin according to any one of claims 1 to 4, **characterized in that** the support layers (4) are formed of a fabric, in which the threads in the longitudinal and transverse directions are the same, but the density of the longitudinal threads per length unit is greater than that of the transverse threads.

7. The diving fin according to any one of the preceding claims, **characterized in that** the number of the inner layers (4) is 3 to 16, preferably 3 to 5.

8. The diving fin according to any one of the preceding claims, **characterized in that** the fin blade (3) is manufactured by the infusion process.

9. The diving fin according to any one of the preceding claims, **characterized in that** the fin blade is formed by a plurality of concave and convex segments (7a, 7b) alternating from the proximal portion to the distal portion of the fin blade, with the crests of the concave and convex segments oriented transverse to the longitudinal direction of the fin blade.

10. The diving fin according to claim 9, **characterized in that** the amplitude of the successive concave and convex segments decreases towards the distal end of the fin blade.

11. The diving fin according to claim 9 or 10, **characterized in that** the wave length of the successive concave and convex segments along the fin blade is equal or decrease towards the distal end of the fin blade.

12. The diving fin according to any of claims 9 to 11, **characterized in that** the distal end of the diving fin is formed flat, i.e. without concave and convex segments.

13. The diving fin according to any one of the preceding claims, **characterized in that** the longitudinal edge of the fin blade is provided with a rubber profile in the form of a wing.

## Patentansprüche

1. Tauchflosse (1), die umfasst:
einen Fußabschnitt (2) und
ein Flossenblatt (3), das an seinem distalen Ende mit dem Fußabschnitt (2) verbunden ist, wobei das Flossenblatt (3) zwei Trägerschichten (4), die entlang der gesamten Länge des Flossenblatts (3) verlaufen, und eine Vielzahl von inneren Schichten (5) zwischen den beiden Trägerschichten (4), die von dem proximalen Ende des Blatts in Richtung zu dem distalen Ende über wenigstens einen Teil der Längsabmessung des Flossenblatts verlaufen, umfasst, wobei jede Trägerschicht (4) und innere Schicht (5) harzimprägnierte Fasern umfasst,
**dadurch gekennzeichnet, dass** wenigstens in den Trägerschichten (4) ein Verhältnis zwischen der Anzahl von im Wesentlichen in der Längsrichtung orientierten Fasern pro Längeneinheit und der Anzahl von im Wesentlichen in der Querrichtung der Tauchflosse orientierten Fasern pro Längeneinheit wenigstens 1,5 beträgt.

2. Tauchflosse nach Anspruch 1, **dadurch gekennzeichnet, dass** das Verhältnis zwischen der Anzahl von in der Längsrichtung orientierten Fasern pro Längeneinheit und der Anzahl von in der Querrichtung der Tauchflosse orientierten Fasern weniger als 9, vorzugsweise 2 bis 4, beträgt.

3. Tauchflosse nach Anspruch 1 oder 2, **dadurch gekennzeichnet, dass** sie ferner zwei Schutzschichten (6) umfasst, die an der Außenseite jeder der Trägerschichten (4) angeordnet sind.

4. Tauchflosse nach einem der vorstehenden Ansprüche, **dadurch gekennzeichnet, dass** die Fasern der Träger- (4) und inneren (5) Schichten ausgewählt sind aus Kohlenstofffasern, Glasfasern oder anderen Fasern mit einem Young's Modul von wenigstens 60 GPa und einer Zugfestigkeit von wenigstens 500 MPa oder Kombinationen davon.

5. Tauchflosse nach einem der vorstehenden Ansprüche, **dadurch gekennzeichnet, dass** die Trägerschichten (4) aus einem Leinwandgewebe gebildet sind, wobei die Fäden in der Längsrichtung eine höhere Anzahl an Fasern aufweisen als die Fäden in der Querrichtung.

6. Tauchflosse nach einem der Ansprüche 1 bis 4, **dadurch gekennzeichnet, dass** die Trägerschichten (4) aus einem Gewebe gebildet sind, bei dem die Fäden in der Längs- und der Querrichtung gleich sind, die Dichte der Längsfäden pro Längeneinheit aber größer ist als jene der Querfäden.

7. Tauchflosse nach einem der vorstehenden Ansprüche, **dadurch gekennzeichnet, dass** die Anzahl der inneren Schichten (4) 3 bis 16, vorzugsweise 3 bis 5, beträgt.

8. Tauchflosse nach einem der vorstehenden Ansprüche, **dadurch gekennzeichnet, dass** das Flossenblatt (3) durch das Infusionsverfahren hergestellt ist.

9. Tauchflosse nach einem der vorstehenden Ansprüche, **dadurch gekennzeichnet, dass** das Flossenblatt durch eine Vielzahl von konkaven und konvexen Segmenten (7a, 7b) gebildet ist, die sich von dem proximalen Abschnitt zu dem distalen Abschnitt des Flossenblatts abwechseln, wobei die Scheitelpunkte der konkaven und konvexen Segmente quer zu der Längsrichtung des Flossenblatts ausgerichtet sind.

10. Tauchflosse nach Anspruch 9, **dadurch gekennzeichnet, dass** die Amplitude der aufeinanderfolgenden konkaven und konvexen Segmente in der Richtung zu dem distalen Ende des Flossenblatts abnimmt.

11. Tauchflosse nach Anspruch 9 oder 10, **dadurch gekennzeichnet, dass** die Wellenlänge der aufeinanderfolgenden konkaven und konvexen Segmente entlang des Flossenblatts in der Richtung zu dem distalen Ende des Flossenblatts gleich bleibt oder abnimmt.

12. Tauchflosse nach einem der Ansprüche 9 bis 11, **dadurch gekennzeichnet, dass** das distale Ende der Tauchflosse flach, d.h. ohne konkave und konvexe Segmente, ausgebildet ist.

13. Tauchflosse nach einem der vorstehenden Ansprüche, **dadurch gekennzeichnet, dass** die Längskante des Flossenblatts mit einem Gummiprofil in der Form eines Flügels versehen ist.

## Revendications

1. Palme de plongée (1) qui comprend :
une partie pied (2) et
une lame de palme (3) reliée à la partie pied (2) à son extrémité distale, la lame de palme (3) comprenant deux couches de support (4) s'étendant sur toute la longueur de la lame de palme (3) et une pluralité de couches internes (5) entre les deux couches de support (4) s'étendant depuis l'extrémité proximale de la lame vers l'extrémité distale sur au moins une partie de la dimension longitudinale de la lame de palme, chaque couche de support (4) et chaque couche interne (5) comprenant des fibres imprégnées de résine,
**caractérisée en ce qu'**au moins dans les couches de support (4), un rapport entre le nombre de fibres par unité de longueur orientées sensiblement dans la direction longitudinale et le nombre de fibres par unité de longueur orientées sensiblement dans la direction transversale de la palme de plongée est d'au moins 1,5.

2. Palme de plongée selon la revendication 1, **caractérisée en ce que** le rapport entre le nombre de fibres par unité de longueur orientées dans la direction longitudinale et le nombre de fibres orientées dans la direction transversale de la palme de plongée est inférieur à 9, de préférence de 2 à 4.

3. Palme de plongée selon la revendication 1 ou 2, **caractérisée en ce qu'**elle comprend en outre deux couches protectrices (6) disposées sur l'extérieur de chacune des couches de support (4).

4. Palme de plongée selon l'une quelconque des revendications précédentes, **caractérisée en ce que** les fibres des couches de support (4) et internes (5) sont choisies parmi les fibres de carbone, les fibres de verre et les autres fibres ayant un module d'Young d'au moins 60 GPa et une résistance à la traction d'au moins 500 MPa, ou les combinaisons de celles-ci.

5. Palme de plongée selon l'une quelconque des revendications précédentes, **caractérisée en ce que** les couches de support (4) sont constituées d'un tissu en armure toile, les fils dans la direction longitudinale ayant un plus grand nombre de fibres que les fils dans la direction transversale.

6. Palme de plongée selon l'une quelconque des revendications 1 à 4, **caractérisée en ce que** les couches de support (4) sont constituées d'un tissu dans lequel les fils dans les directions longitudinale et transversale sont identiques, mais la densité des fils longitudinaux par unité de longueur est supérieure à celle des fils transversaux.

7. Palme de plongée selon l'une quelconque des revendications précédentes, **caractérisée en ce que** le nombre des couches internes (4) est de 3 à 16, de préférence de 3 à 5.

8. Palme de plongée selon l'une quelconque des revendications précédentes, **caractérisée en ce que** la lame de palme (3) est fabriquée par le procédé d'infusion.

9. Palme de plongée selon l'une quelconque des revendications précédentes, **caractérisée en ce que** la lame de palme est formée par une pluralité de segments concaves et convexes (7a, 7b) alternant de la partie proximale à la partie distale de la lame de palme, avec les sommets des segments concaves et convexes orientés transversalement à la direction longitudinale de la lame de palme.

10. Palme de plongée selon la revendication 9, **caractérisée en ce que** l'amplitude des segments concaves et convexes successifs diminue vers l'extrémité distale de la lame de palme.

11. Palme de plongée selon la revendication 9 ou 10, **caractérisée en ce que** la longueur d'onde des segments concaves et convexes successifs le long de la lame de palme est égale ou décroissante vers l'extrémité distale de la lame de palme.

12. Palme de plongée selon l'une quelconque des revendications 9 à 11, **caractérisée en ce que** l'extrémité distale de la palme de plongée est formée plate, c.-à-d. sans segments concaves et convexes.

13. Palme de plongée selon l'une quelconque des revendications précédentes, **caractérisée en ce que** le bord longitudinal de la lame de palme est pourvu d'un profilé en caoutchouc prenant la forme d'une aile.
